

June 4, 1935.

D. J. CAMPBELL

2,004,061

COMPOSITE BRAKE DRUM

Filed Nov. 13, 1933



INVENTOR

Donald J. Campbell

By Leirance & Van Autreby

ATTORNEYS

## UNITED STATES PATENT OFFICE

2,004,061

## COMPOSITE BRAKE DRUM

Donald J. Campbell, Spring Lake Township, Ottawa County, Mich., assignor to Campbell, Wyant & Cannon Foundry Company, Muskegon, Mich., a corporation of Michigan

Application November 13, 1933, Serial No. 697,817

4 Claims. (Cl. 22—203)

This method relates to a brake drum and also to its method of manufacture.

One object of the invention is to more easily and thoroughly join an iron of an alloyed compound 5 position braking band to a steel or other thin metal supporting shell than has been heretofore accomplished.

The invention consists in producing a supporting shell, heating the shell sufficiently to prevent 10 chilling of molten copper, revolving the shell slowly in a suitable mechanism, depositing into the shell a measured quantity of molten iron that has been alloyed with copper, increasing the rate of rotation while the iron is in a molten state 15 until a sufficient quantity of the copper is driven to the inner peripheral surface of the shell and separates the molten iron from the shell by a thin layer of copper, the copper being joined to the shell and to the iron as by fusion.

20 The invention is carried out by the mechanism disclosed in the accompanying drawing, in which:

Fig. 1 is a sectional view of a mechanism for revolving the shell and depositing of the metal 25 in the shell.

Fig. 2 is a sectional view of a brake drum produced by the invention.

While a mechanism is illustrated by the mechanism of the drawing, it is understood that the 30 invention is not confined to any distinct mechanism.

Similar characters of reference refer to similar parts throughout the several views of the drawing.

35 Referring to Fig. 1, numeral 10 indicates a chuck housing which receives jaws 11, such jaws being shown in contracted position but capable of being extended outwardly relative to the housing 10 whereupon they are expanded and release 40 the brake drum held therein. The chuck housing 10 is located in suitable bearings, one of which is indicated at 12, whereby it may be properly rotated.

45 Referring now particularly to Fig. 2, numeral 13 indicates a shell, preferably formed of sheet steel, having a cast iron liner 14 therein. A layer of copper or copper alloy 15 is positioned between the cast iron shell 14 and the steel supporting member 13.

50 In carrying out the invention it is desirable to first melt the iron in a cupola, transfer it to an electric furnace and introduce the desired quantity of copper and other alloys and where 55 the whole mass of iron and alloys is brought to

the desired temperature for depositing into the revolving heated shell. It has been found that the quantity of copper may vary between 2 percent and 10 percent and in some cases even more, but for good results a percentage of 4 percent. 5 The temperature in cupolas in which cast iron is melted for foundry purposes is seldom if ever below 2400° F. and with so-called hot blast furnaces may reach 2600° F. Therefore, to those skilled in foundry practice it is well known that 10 cupola melted iron is at approximately 2400 to 2600° F. and that a transfer to an electric furnace would be to either elevate such temperature or maintain it as high as initially produced while the copper is melting and disseminating there- 15 through.

It will be appreciated that copper is of greater density than the cast iron and thus during the rotation of the shell, the molten copper will flow outwardly due to centrifugal force and contact 20 against the inner side of the steel shell 13. Thus the copper will be positioned exteriorly of the cast iron braking drum. Also, copper is a much better conductor of heat than cast iron and thus the outer oil shell will be more easily fused in its 25 inner side.

There is produced a composite brake drum structure having an outer steel shell, an inner wearing band of cast iron through which part 30 of the copper used may be disseminated and a 35 layer or film of copper between the cast iron and steel. There is an intimate and continuous joinder of the cast iron to the steel by means of the intermediate copper which has all of the 40 effects and characteristics of a complete and continuous brazing connection of the cast iron to the steel and by means of which fully as intimate a connection of the cast iron to the steel is made as if the cast iron was fused thereto. At the same time the copper adds strength and 45 toughness to the cast iron liner and also at the binding band between the cast iron and steel adds strength to the steel outer shell.

It is to be understood that my invention is not 45 definitely limited to the metals herein recited as obviously each of these metals might be replaced by others having somewhat like characteristics.

The invention is defined in the appended claims.

I claim:

1. The method of producing a brake drum which consists in providing a shell, melting a quantity of cast iron in a cupola, transferring it to an electric furnace and then introducing between 3% and 10% of copper thereto, rotating 55

the shell, depositing the molten mixture within the shell while the shell is rotating and then cooling the mixture.

2. The method of manufacturing a brake drum which consists in providing a steel shell, inserting a molten mixture of cast iron and copper therein, the copper not exceeding ten percent of the mass of iron and also being at least three percent thereof, and then rotating the shell at 10 such a speed as to cause an appreciable separation of the metals due to the action of centrifugal force thereon and then cooling the several elements.

3. The method of manufacturing a brake drum which consists in providing a steel shell, rotating

the shell, introducing molten copper and molten cast iron into the shell either before or after the start of its rotation, the rotation being of sufficient speed to cause partial segregation of the metals and then cooling the metals, said copper content being between 3 and 10 percent.

4. The method of manufacturing brake drums which consists in providing a steel shell, rotating the steel shell, introducing into the steel shell while it is rotating, molten iron and copper, then rotating the said shell, iron and copper at a speed sufficient to cause separation of copper from the iron to form a film of copper between the steel shell and the iron.

DONALD J. CAMPBELL 15